

April 23, 1929.

H. EWALD

1,710,303

METHOD OF PRODUCING PHOTOGRAPHIC PROCESS SCREENS

Original Filed Jan. 15, 1923



FIG. 1



FIG. 2

INVENTOR:  
Herman Ewald

By  
Jones, Addington, Ames + Siebold  
ATTYS.

## UNITED STATES PATENT OFFICE.

HERMAN EWALD, OF CHICAGO, ILLINOIS.

## METHOD OF PRODUCING PHOTOGRAPHIC-PROCESS SCREENS.

Application filed January 15, 1923, Serial No. 612,797. Renewed May 11, 1928.

My invention relates to a color separation process screen, and to a photographic process for the natural reproduction of oil paintings, water-color sketches, machinery, or natural scenes and the like.

In a general way my invention contemplates the reproduction of an original by the use of a screen provided with an irregularly wrinkled or corrugated coating.

10 The screen effect is accomplished by the texture which is high at the crest of the corrugation and deep between the corrugations, the deeper part between the corrugations having the effect of a dark portion of the screen 15 and the higher part at the crest of the corrugation having the effect of a transparent portion. The effect of this screen on the negative is to give it an irregular open natural transparent effect, makes the details stand out 20 much more clearly and more like the original than would be possible with the old half-tone screen.

I also place the color directly in the surface of the screen, and place the screen directly in 25 front of the sensitized dry plate. My invention contemplates particularly a close contact illumination of the sensitized plate by a colored plate, which colored plate may also have a screen texture, although it is obvious 30 that two separate plates may be employed, one being the color plate and the other the texture screen, or that a plate may be provided having a color screen on one side and a texture screen on the other. My method is so 35 simple to use, that any photographer can easily get good results in color reproduction without much experience in handling the screen.

In reproducing an original in colors, all 40 that is necessary to do is to use four of my screens of the proper color, making one negative from each screen, and then use these negatives without any retouching to make a corresponding number of zinc etchings, from 45 which the final reproduction is printed.

In printing the final reproduction, I use a flat coated material to receive the colors, such as metal or specially prepared paper or canvas which holds the colors on top of the 50 surface so that they do not sink flat but stand up bright and strong, so that in the reproduction, for instance, of an oil painting, the effect is strikingly similar to the oil painting itself, having the appearance of brush work

done by an artist in oil or water-color and 55 pastel.

The main inventive idea is in the color screen itself, and in the method by which it is reproduced.

In the drawings—

Fig. 1 is a greatly enlarged plan view of a fragment of the color screen, showing the wrinkled or corrugated coating; and

Fig. 2 is a section on the line 2—2 of Fig. 1.

In making my new screen, I use a glass 60 plate 10 which is perfectly even on the surface, and coat the same with a specially prepared gelatine emulsion which is sensitized to light, when dried on the glass. This emulsion may be prepared as follows: 5 oz. of best hard 70 clear gelatine are diluted in 10 oz. of distilled water, and one oz. of finely powdered potassium bichromate is diluted in the gelatine and water at a temperature not over 120 degrees F. Two oz. of ammonia water is then added 75 and the mixture is filtered three or four times through a felt filter. After this solution is filtered it is poured warm onto a warm glass plate so that the solution can run easily all over the surface of the glass. This glass 80 plate is then set in a dry oven with its coated surface level, and is dried at a temperature of about 90 degrees F. for about 2 hours.

This dry coated plate which is now sensitive to the light, is then exposed to a light 85 (either to the sun or to artificial light) for a short time, as long as is necessary, depending upon the power of the light. This hardens the emulsion on the glass plate.

After the plate has been exposed to the 90 light for a certain time, as long as needed, it is placed in a 25% acetic acid bath which causes the surface of the exposed emulsion to become irregularly wrinkled or corrugated, the corrugations or wrinkles being discontinuous, 95 and the surface having an appearance under a magnifying glass as though it were thickly sprinkled with small worms as indicated at 11.

The plate may be exposed to the action of this acetic acid bath for about 5 minutes, after 100 which it is washed out for about an hour in running water. After it has been washed, it is cleared out in a bath of alum and citric acid, which makes the plate more transparent.

After the plate has thus been washed and 105 cleared, it is placed in an acetic acid bath which is diluted with proper aniline dye colors which will soak into the emulsion coating

on the glass plate, giving this coating the desired color.

After the screen has thus been colored, it is dried in a dry room under a low temperature 5 not over 80 degrees F. the drying being best accomplished by cool air ventilation.

After the plate is thus colored and dyed, the emulsion screen surface is coated with a clear special transparent water-proof varnish 10 which makes the emulsion coating more clear and transparent and water-proof, and keeps the colors in the gelatine surface protected from damp atmosphere which would make the screen filmy and destroy the clear transparent 15 effect.

The use of the plate has been outlined above. As previously stated, if the four color process is to be used, four of my screens of proper color are prepared, a negative is made from 20 each screen, and these negatives are then used without retouching to make the corresponding number of zinc etchings from which the final reproduction is printed.

Having thus described my invention, what 25 I claim as new and desire to secure by United States Letters Patent is:

1. A method of making a photographic process screen, comprising coating a glass plate with a sensitized gelatine composition 30 which hardens on exposure to light, drying the coating, exposing the coating to the light to harden it and subjecting the coating to a 25% acetic acid bath, to cause the surface of the coating to become irregularly corrugated.

35 2. A method of making a photographic process screen, comprising coating a glass plate with a sensitized gelatine composition which hardens on exposure to light, drying the coating, exposing the coating to the light 40 to harden it and subjecting the coating to a

25% acetic acid bath for about 5 minutes, to cause the surface of the coating to become irregularly corrugated.

3. A method of making a photographic process screen, comprising coating a glass 45 plate with a composition of about 5 oz. of clear gelatine diluted with 10 oz. of distilled water, 1 oz. of potassium bichromate and 2 oz. of ammonia water, drying the coating at a temperature of about 90 degrees F. for about 2 50 hours, exposing the coating to light for a short time to harden it, subjecting the coating to a 25% acetic acid bath to cause the surface of the coating to become irregularly corrugated, washing off the plate for about an 55 hour in water, and subjecting the washed plate to a bath of alum and citric acid to clear it out and make more transparent.

4. A method of making a photographic process screen, comprising coating a glass 60 plate with a composition of about 5 oz. of clear gelatine diluted with 10 oz. of distilled water, 1 oz. of potassium bichromate and 2 oz. of ammonia water, drying the coating at a temperature of about 90 degrees F. for about 65 2 hours, exposing the coating to light for a short time to harden it, subjecting the coating to a 25% acetic acid bath to cause the surface of the coating to become irregularly corrugated, washing off the plate for about an hour 70 in water, subjecting the washed plate to a bath of alum and citric acid to clear it out and make more transparent, and placing the washed and cleared out plate in an acetic acid bath diluted with dye-color which will soak 75 into the coating to give it the proper color.

In witness whereof, I have hereunto subscribed my name.

HERMAN EWALD.